

## UNITED STATES PATENT OFFICE.

ERNST JOHANSEN, OF FALL RIVER, MASSACHUSETTS, ASSIGNOR TO NEW ENGLAND OIL REFINING COMPANY, OF FALL RIVER, MASSACHUSETTS, A CORPORATION OF MASSACHUSETTS.

## MOTOR FUEL AND ITS MANUFACTURE.

No Drawing.

Application filed April 4, 1924. Serial No. 704,165.

This invention relates to a novel fuel for use in internal combustion engines.

It has been known for some time that certain organic metallic compounds, especially 5 lead compounds, when added to motor fuels, such as certain commercial gasolines, render the vapors of the latter when mixed with air capable of much higher compression, than would otherwise be the case, before the mixture 10 will detonate when ignited under pressure. In other words, by the use of gasoline thus treated, internal combustion motors can be run at a much higher compression than in the case of gasoline not so 15 treated without the occurrence of the objectionable phenomenon known as "knocking," thus greatly increasing the power and efficiency of the engine.

The lead compounds heretofore used for 20 this purpose are organic lead compounds produced by special synthetic processes widely differing from those employed in the refining of petroleum. The expense of producing these organic lead compounds is relatively 25 high so that the price of the fuels to which these compounds have been added is considerably increased.

I have found that motor fuels containing 30 organic metallic compounds may be readily and cheaply produced by the direct action of certain metallic oxides or compounds upon certain petroleum products. In this way, the desirable metal compounds are formed directly in the petroleum product or 35 fuel and remain dissolved in the latter. The costly separate production of expensive synthetic metal compounds and their addition to the motor fuel, such as gasoline, are thus avoided.

40 In preparing my novel fuel I use the petroleum products known as "sour distillates," (see Das Erdöl by Engler, Hofer, 1911, vol. 3, page 871, foot note), obtained in the distillation of crude petroleum or intermediate petroleum products. These distillates are characterized by their ability to react with certain metallic compounds, for example certain metallic oxides or a solution of said oxides in an alkali solution, thereby 45 forming metallic compounds that will remain dissolved in the distillates. I expose these distillates to the action of said metallic compounds or oxides, preferably using for this purpose either lead oxide or

alkali plumbite, but do not limit myself to the use of these materials. A fraction of sour distillate, having a boiling range suitable for motor fuel, is first freed from the 55 elementary sulphur therein contained in any suitable manner, for instance by redistillation. Previous to this or after, the distillate may be treated with a slight amount of sulphuric acid to improve the color and odor 60 of the distillate, following this by washing with water. This however is optional. The product obtained by the redistillation 65 is then agitated at ordinary temperature with lead oxide (litharge) either in dry form or dissolved in a solution of sodium or potassium hydroxide whereby a sodium or 70 potassium plumbite is formed (alkali plumbite). The color of the distillate, which is generally water white, is by this treatment 75 changed to yellow. If the dry lead oxide is used, any excess of lead oxide is first allowed to settle, whereupon the liquid product becomes perfectly clear and can be drawn off ready for use. If a solution of lead oxide in sodium or potassium hydroxide is used any excess thereof will separate 80 and having been allowed to settle may be drawn off. I preferably use from one to three pounds of lead oxide per forty-two gallon barrel of distillate.

The clear settled yellow product containing 85 up to one gram of lead per liter, or even more, is permanent under ordinary conditions, and can be used as a motor fuel for engines working with high compression. It can be used either pure or blended in any 90 suitable proportions with gasoline or other motor fuels, such as benzol, alcohol or ether.

The novel motor fuel produced by the above method is believed to contain the lead in the form of addition compounds. The 95 advantages of the novel fuel, besides those already mentioned, are low cost of production and simple manner of preparation, requiring no other apparatus or reagents than those universally used in the refining of 100 petroleum products.

## Claims:

1. A motor fuel which comprises a solution in petroleum hydrocarbons of compounds of a metallic oxide with sour distillate components, said compounds being soluble in said fuel.
2. A motor fuel which comprises a solu-

tion in petroleum hydrocarbons of compounds of lead with sour distillate components.

3. A motor fuel which comprises a solution in petroleum hydrocarbons of compounds of lead oxide with sour distillate components.

4. A motor fuel which comprises a solution in petroleum hydrocarbons of metal compounds with sour distillate components,

said compounds being soluble in said fuel.

5. A motor fuel which comprises a solution in petroleum hydrocarbons of lead oxide compounds with sour distillate components and containing up to one gram of lead per liter of fuel.

In testimony whereof, I have signed my name to this specification.

ERNST JOHANSEN.